

Nov. 22, 1960

L. PÉRAS

2,961,563

SLIPPING-SPARK IGNITION PLUGS

Filed April 1, 1958



1

2,961,563

## SLIPPING-SPARK IGNITION PLUGS

Lucien Péras, Billancourt, France, assignor to Régie Nationale des Usines Renault, Billancourt, France

Filed Apr. 1, 1958, Ser. No. 725,710

Claims priority, application France Apr. 24, 1957

3 Claims. (Cl. 313—131)

This invention relates in general to spark ignition devices and more particularly to spark plugs of the type wherein the spark is produced by discharging a capacity and wherein the electrical voltage or tension and the electrode gap have such values that the spark cannot take place in the atmosphere where the ignition is required unless this spark remains in contact with a solid insulating member disposed between the electrodes. In the absence of such solid insulating member the spark will not fly unless a considerably higher tension is used and in this case either the advantages resulting from capacity-discharge ignition must be waived or the inter-electrode gap must be set at a very small value of the order of 0.008" to 0.002"; now it is evident that this condition is rather difficult to meet, and furthermore as a consequence of the electrode wear caused by sparks recurring at a high rate the interelectrode gap would rapidly increase to a value preventing the passage of sparks.

It is already known, in their application to internal combustion engines, to constitute spark plugs the sparking element of which consists of two electrodes spaced about 0.004" to 0.008" apart, the inter-electrode gap being occupied by a solid-supporting insulator flush with the electrode surfaces. However, the useful life of capacity discharge spark plugs of this character is reduced more or less by two main and different causes, namely:

Electrode wear, whereby the relative spacing of the sparking edges increases until it is too great to enable the spark to fly between these edges;

Premature wear of the insulator due to the thermal action exerted thereon by the sparks, whereby the sparks will progressively "sink" inside the cartridge until they become unable to ignite the fuel mixture.

Now according to this invention it is possible to provide capacity-discharge spark plugs characterized by an extremely long useful life.

This invention provides a method of manufacturing spark plugs of the type defined hereinabove, wherein the insulator disposed between the electrodes is rendered particularly apt to facilitate in a reliable and lasting manner the passage of sparks by being coated with an enamel of special composition which has a high specific inductive capacity.

According to a typical form of embodiment of the invention, the insulator, whether cured or uncured, consisting for example of sintered alumina or clay-bound alumina, is coated on its face turned towards the chamber containing the fuel mixture to be ignited, with an enamel applied with a brush, by dipping or by any other adequate means, this enamel consisting of a suspension in a liquid of the material in a finely divided state. After the coating step, the insulator is dried and brought to the proper baking temperature in a suitable atmosphere.

Thus, after fitting the insulator in the assembly, a spark plug for capacity-discharge ignition which has an insulator of adequate shape, enamelled on its operative portion, that is, on the portion situated in the inter-

2

electrode gap on which the sparks are caused to fly and slip, is obtained. The insulator to be coated with the aforesaid enamel may have the following composition:

|   |                                | Percent  |
|---|--------------------------------|----------|
| 5 | Al <sub>2</sub> O <sub>3</sub> | 55 to 95 |
|   | SiO <sub>2</sub>               | 5 to 45  |
|   | TiO <sub>2</sub>               | 0 to 1   |
|   | CaO                            | 0 to 5   |

10 An enamel composition particularly suitable for coating the active surface of an insulator of the kind defined hereinabove has the following composition:

|    |                                            |
|----|--------------------------------------------|
| 15 | 5% < TiO <sub>2</sub> < 30%                |
|    | 20% < BaO < 46%                            |
|    | 1% < B <sub>2</sub> O <sub>3</sub> < 10%   |
|    | 30% < SiO <sub>2</sub> < 45%               |
| 20 | 0.5% < Al <sub>2</sub> O <sub>3</sub> < 3% |
|    | 1% < Na <sub>2</sub> O < 9%                |

In this enamel the last four elements associated beforehand by baking are in a vitreous condition. The oxides of titanium and barium, or barium titanate are thoroughly mixed by crushing the vitreous phase until a finely divided powder is obtained. This powder in the form of an aqueous suspension is then applied by means of a brush on the portion of the aluminous insulator which is to be enamelled. After drying, the coated insulator is brought to the curing temperature of 800° to 1,350° C., this curing operation being effected compulsorily in a reducing atmosphere, for example of hydrogen; the enamel is obtained to the proper degree when its color is dark blue and adheres perfectly on its aluminous support.

The baking of the enamel may be carried out by means of a heating torch successively in the oxidizing or reducing portion of the flame, or by using any other adequate heating means of which at least the last phase is a reducing one.

Satisfactory results are also obtained by carrying out the last heating step in a nitriding atmosphere.

An ignition spark plug of the slipping-spark type according to this invention is illustrated diagrammatically 45 by way of example in the single figure of the attached drawing. In this figure, the reference numeral 1 is the insulator, 2 and 3 are the electrodes, and 4 the enamel coating.

I claim:

50 1. A slipping-spark ignition spark plug having an insulator interposed between electrodes, the active portion of said insulator being coated with a baked enamel having a high specific inductive capacity, said enamel being the non-volatile residue of an aqueous suspension of the enamel components in a finely-divided state, said enamel consisting essentially of 5 to 30% TiO<sub>2</sub>, 20 to 46% BaO, 1 to 10% B<sub>2</sub>O<sub>3</sub>, 30 to 45% SiO<sub>2</sub>, 0.5 to 3% Al<sub>2</sub>O<sub>3</sub> and 1 to 9% Na<sub>2</sub>O.

60 2. A method of manufacturing spark plugs of the type wherein a slipping-spark is produced in contact with a solid insulator, wherein the insulator interposed between the electrodes of the spark plug is rendered particularly suitable for the passage of the sparks, which comprises the steps of coating the active portion of said insulator with an enamel having a high specific inductive capacity, said enamel being applied as an aqueous suspension of its components in a finely divided state, drying the insulator and baking the enamel coating upon said insulator in a reducing or nitriding atmosphere at a temperature of 800 to 1350° C., said enamel consisting essentially of 5 to 30% TiO<sub>2</sub>, 20 to 46% BaO, 1 to 10%

70

$B_2O_3$ , 30 to 45%  $SiO_2$ , 0.5 to 3%  $Al_2O_3$  and 1 to 9%  $NaO_2$ .

3. A method of manufacturing spark plugs of the type wherein a slipping-spark is produced in contact with a solid insulator, wherein the insulator interposed between the electrodes of the spark plug is rendered particularly suitable for the passage of the sparks, which comprises the steps of coating the active portion of said insulator with an enamel having a high specific inductive capacity, said enamel being applied as an aqueous suspension of its components in a finely-divided state, drying the insulator and baking the enamel coating upon said insulator in a suitable atmosphere, said enamel consisting essen-

tially of 5 to 30%  $TiO_2$ , 20 to 46%  $BaO$ , 1 to 10%  $B_2O_3$ , 30 to 45%  $SiO_2$ , 0.5 to 3%  $Al_2O_3$  and 1 to 9%  $NaO_2$ .

4  
References Cited in the file of this patent

## UNITED STATES PATENTS

|           |          |       |               |
|-----------|----------|-------|---------------|
| 1,123,017 | Schroter | ----- | Dec. 29, 1914 |
| 2,010,776 | Frost    | ----- | Aug. 6, 1935  |
| 2,527,884 | Kaufmann | ----- | Oct. 31, 1950 |
| 2,587,916 | Squier   | ----- | Mar. 4, 1952  |
| 2,715,593 | Clark    | ----- | Aug. 16, 1955 |
| 2,790,104 | Smits    | ----- | Apr. 23, 1957 |